

## UNITED STATES PATENT OFFICE

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MASSACHUSETTS

## BOX TOE

No Drawing. Original application filed October 31, 1922, Serial No. 598,314. Divided and this application filed September 27, 1924. Serial No. 740,414.

This invention has for its object to produce a shoe stiffener or sheet material from which such stiffeners may be produced.

Heretofore it has been customary in the manufacture of shoe stiffeners such as box toes to form a sheet of fibrous material, usually cotton and wool felt or like open porous material, and then to saturate or impregnate the sheet with a molten mass of a stiffening agent in the nature of hydrocarbons, which when cold is hard and friable but which when softened by a relatively moderate degree of heat permits the sheet or blank cut therefrom to become limp and flexible, so that the box-toe blank may be molded about the end of the last in pulling over or lasting the shoe. Various stiffening agents have been employed for this purpose, such as resins, gums, asphalts and hydrocarbons of the nature of Montan wax.

More particularly, the object of the present invention is to produce box toes or the sheets from which the box-toe blanks may be cut, by incorporating the stiffening agent with the pulp before manufacture into a sheet on a paper machine so as to render unnecessary the step of separately impregnating the already formed sheet of fibrous material. It is necessary that the stiffening agent or agents should be thoroughly distributed throughout the sheet, that they should be of such nature that the box toe when molded is resilient and stiff, that they may be softened so as to render the sheet limp and flexible when heated to a relatively low temperature, and that they will set quickly when permitted to cool. One of the prime requisites of the sheet is that it must not part or tear easily when the stiffening agent is in a soft plastic condition, and that it may be stretched to some extent and pulled about the toe end of the last without being weakened or torn so as to conform to the shape of the last without injury.

The present invention consists of a box-toe blank, the sheet from which it is cut and a method of producing the same which will provide a box toe having the optimum characteristics which I have hereinbefore referred to.

In initially preparing the sheet, I employ

a furnish, including long fibers such as cattle hair, long rope fibers or flax fibers, and even in some cases may utilize long cotton fibers. In addition to these fibers, however, I also employ short fibers, preferably of the character of wood pulp used in the manufacture of paper,—this for the reason that a sheet formed only of long fiber is too open and porous and requires some shorter fiber in order to secure the necessary felting in the formation of the sheet on the paper machine. Inasmuch as an object which I desire to achieve is to secure a maximum quantity of stiffening agent in the sheet, it is necessary that the fibrous body of which the sheet is formed should be of such character that it will form properly in a web and yet be sufficiently open to permit the proper discharge of the water from the cylinder in the paper machine. An even web formation is secured by employing both the long fibers of the nature of cattle hair and short fibers such as obtained in the production of chemical wood pulp or such as obtained from waste kraft paper or the like. Of course, in lieu of wood pulp, one might employ rags or other raw material which provides relatively short fibers, which, when mixed with long fibers, will furnish a sheet having the desired characteristics.

As the stiffening agent I may utilize any gums or bituminous materials such as rosin, asphalt, Montan wax, copal or the like, which will give to the box toe the necessary stiffness and resiliency, and which will soften at a relatively low degree of heat and set quickly when cooled. Normally adhesive bituminous materials may likewise be utilized for furnishing the stiffening agents, provided they be in the form of an aqueous emulsion, so that they may be diluted with water and be thoroughly incorporated with the other elements or ingredients of the furnish in the beater stock.

As an example, one may proceed as follows: 8 parts by weight of cattle hair or other long fibers and 8 parts by weight of sulphate pulp or equivalent short fibrous material may be placed in the beater with a large amount of water, much more than is ordi-

narily necessary for beating the stock. The beating engine is started in operation but the knives are carefully adjusted so as not to cut the fibers but merely to brush them and secure a thorough, physically homogeneous mixture. The stock should be thinned with water as this permits the rapid admixture of the ingredients. Of course, by taking a longer time, one might secure the same results with a thicker stock or one having less water. By having a very thin stock, it is possible to secure the desired physical homogeneity in the course of 15 to 30 minutes. After the beater contents have been brushed as described, the thermo-plastic stiffening agents may now be added. In the example herein given, I employ 35 parts by weight of rosin, 25 parts by weight of gilsonite and 5 parts by weight of Montan wax, all pulverized to about 40 mesh. These ingredients are introduced into the beater, together with about 30 parts of asphalt emulsified or dispersed in water. This emulsion or dispersion preferably consists of normally adhesive asphalt emulsified or dispersed in water with a colloidal clay emulsifying agent, the asphalt constituting the disperse phase of the emulsion. The amount of the emulsion added to the beaters is figured as the asphalt on a dry basis. An emulsion, such as herein described, is not per se my invention, and can be obtained on open market under the trade name of "K-B" emulsion.

With these hydrocarbon resinous ingredients, which constitute the thermo-plastic stiffening agent, I preferably add a small amount of casein dissolved in an alkaline solution. Instead of casein, I may use any other ingredient, which when precipitated by a precipitating agent carries down with it the stiffening materials in a more or less conglomerate mass. Thus, in lieu of casein, I may use rosin size, viscous animal size, or other equivalent material. In some cases, however, I do not utilize either casein or the sizing material last referred to, but ordinarily I find that it may be used with advantage. After these ingredients have been thoroughly intermixed with the fibrous material in the beater by continued rotation of the beater roll adjusted somewhat away from the bed plate, I then add 10 parts by weight of alum as a precipitating agent. The fibrous stock with the stiffening agent thoroughly incorporated therein is now formed into a sheet by a cylinder paper machine, and, when the sheet is of the desired thickness, it is cut and removed from the make-up roll. The sheet is then dried for the removal of water; and, when dry, is relatively open, free and porous with free rosin, gilsonite, Montain wax and asphalt distributed as discrete particles throughout the sheet, and, when magnified, are visible as such.

While still warm from the drier, the sheet is

now preferably passed through calender rolls heated to a sufficient temperature to flux the hydrocarbon stiffening agents so that they will coalesce throughout the sheet. The effect of the calendering is further to condense and compact the sheet, so that, when the sheet cools, it is relatively hard, compact or dense, stiff and resilient; and it is not affected by body temperature or materially affected by solar heat, but may be rendered limp and flexible at a temperature of 140° to 150° F.

It is quite evident that the particular ingredients, which I have mentioned in the foregoing example, may be changed or added to, although the furnish as described gives excellent results. For example, I may change the fibrous ingredients by utilizing 5 parts by weight of long fibers such as cattle hair, 5 parts by weight of sulphate pulp, and 5 parts by weight of the waste of the final sheet or waste which is produced from box-toe material as ordinarily made. In such case, the box-toe waste, which is the residue after cutting out the box toes or other shoe stiffeners, must be disintegrated before being added to the beater. I find that this disintegration may be accomplished by subjecting the material to the action of an Abbe rotary cutter or grinder. Such machines are on the market and are easily procurable. Since there is some tendency of the stiffening agents in the waste to gum the knives, I employ as a preventative a small amount of talc which may be thrown into the grinder from time to time by the handful. For example, I find that in any given amount of the disintegrated waste fiber, there need not be over 1/2% of talc to insure the successful operation of the grinder. The disintegrated waste material consists of the usual fibers of which the felt was formed together with the gums or solid hydrocarbons with which it was impregnated. It is possible to reduce the proportion of the asphalt emulsion from 30 parts by weight to, say, 20 parts by weight, and to increase the percentage of the casein or other size which is employed.

By long continued experiment, I have found that a sheet, having only the asphalt emulsion as the stiffening agent, does not produce satisfactory box toes, for the reason that the sheet is too soft and does not possess the requisite rigidity and resiliency when cold, and that further it becomes too limp and soft when heated in the usual heaters employed in shoe factories in connection with the pulling and lasting operations. I regard however, the employment of the asphalt emulsion as desirable for the reason that the normally adhesive asphalt imparts a certain desirable toughness to the sheet when it is warm, and contributes towards permitting the box-toe blanks to be folded and stretched about the last when the shoe is be-

ing pulled over or lasted. Since the asphaltic emulsion is insufficient to produce a sheet of the necessary resiliency, rigidity and stiffness, I employ rosin, gilsonite or the equivalent which is distributed in the pulp in fine particles. In fact, instead of utilizing both 5 rosin and gilsonite, I may employ rosin alone, although I do not regard the final product as desirable as one in which these 10 two ingredients are employed. Gilsonite having a high melting point, adds stiffness and rigidity to the molded box toe when subjected to body or solar heat. Inasmuch as the hydrocarbons must coalesce and become 15 more or less amalgamated in the sheet, I use a certain proportion of Montan wax, which, because of its high degree of penetrability when molten, acts as a fluxing agent for the other hydrocarbons in the sheet. The addition 20 of Montan wax or like hydrocarbon of high penetrability and relatively low melting point is particularly desirable when a tempering agent such as gilsonite is employed, as otherwise it may be necessary to 25 heat the calendering rolls to such a high temperature to flux or coalesce the other hydrocarbon ingredients as might or would tend to burn the hair or other long fibers employed in making the sheet. An advantage in employing 30 casein rather than other size is that when precipitated with alum it is not affected by dry heat but will soften when moist. Ordinarily, in the pulling over or lasting of 35 shoes, in which stiffened box-toe blanks are employed, it is customary to subject the blank to moist heat, and therefore it is desirable to use some agent which when precipitated is not affected by dry heat but which will soften when subjected to heat and moisture. 40

After the sheet is finished, the blanks are cut and skived to serve as shoe stiffeners, such as box toes or counters.

The stiffening agents may be referred to as 45 thermo-plastic material, meaning to include by that term those compounds or mixtures which function as herein set forth,—namely those which may be incorporated in the wet 50 mass of fibrous material while in a finely divided condition, which soften on the application of heat not injurious to the shoe, which set rapidly when cooled, which give rigidity, stiffness and resiliency to the molded box toe, and which will permit the heated and limp 55 box-toe blank to be stretched about the toe end of the last, in the pulling-over and end-lasting operations.

This is a division of my application Serial No. 598,214 filed Oct. 31, 1922, which has 60 matured into Patent No. 1,544,813, granted July 7, 1925.

What I claim is:

1. A dense, hard and resilient box toe comprising a layer of felted fibers and a thermoplastic material precipitated upon and ad-

herent to the fibers thereof, the content of thermoplastic material in said box toe being in excess of the weight of the fibers, so that said box toe is capable of being made limp by moderate heat and of setting rapidly when cooled. 70

2. A dense, hard and resilient box toe comprising a flat layer of felted fibers having incorporated in and distributed throughout the layer a thermoplastic compound and a precipitate for said compound, the content of thermoplastic compound in said box toe being sufficiently high so that it is capable of being made limp by moderate heat and of setting rapidly when cooled. 75

3. A dense, hard and resilient box toe comprising a flat layer of felted fibers having incorporated in and distributed throughout the layer a thermoplastic compound and a precipitate for said compound, said compound being in a state of coalescence throughout the said layer and being present in amount sufficient so that said box toe is capable of being made limp by moderate heat and of setting rapidly when cooled. 80

4. A hard dense compact resilient box toe consisting of felted fibers, a thermo-plastic stiffening compound in amount in excess of the weight of the fibers so as to render said box toe capable of being made limp by moderate heat, and a precipitate, said fibers comprising both long and short fibers, so that when said box toe is heated it may be stretched about the toe of a last without tearing, said thermo-plastic stiffening compound being of a character to soften at low heat and to set rapidly when cooled, and said precipitate being of such character as to soften when subjected to heat and moisture. 90

5. A dense, hard and resilient box toe, comprising a sheet composed of interfelted fibers, and thermoplastic material preponderating in amount over such fibers precipitated upon and adherent thereto and present in amount sufficient so that said box toe is capable of being made limp by moderate heat and of setting rapidly when cooled. 100

6. A dense, hard and resilient box toe, comprising a sheet composed of long and short fibers interfelted in approximately 115 equal proportions, and thermoplastic material preponderating in amount over such fibers precipitated upon and adherent thereto and present in amount sufficient so that said box toe is capable of being made limp by 120 moderate heat and of setting rapidly when cooled.

In testimony whereof I have affixed my signature.

ALBERT L. CLAPP. 125